

A. W. H. LENDERS.  
SIZE AND PROCESS OF MAKING SAME.  
APPLICATION FILED JULY 8, 1916.

1,253,397.

Patented Jan. 15, 1918.



INVENTOR

Adolf W. H. Lenders  
BY  
Barnett Johnson  
ATTORNEY S.

# UNITED STATES PATENT OFFICE.

ADOLPH W. H. LENDERS, OF CEDAR RAPIDS, IOWA.

## SIZE AND PROCESS OF MAKING SAME.

1,253,397.

Specification of Letters Patent. Patented Jan. 15, 1918.

Application filed July 8, 1916. Serial No. 108,188.

*To all whom it may concern:*

Be it known that I, ADOLPH W. H. LENDERS, a citizen of the United States, residing at Cedar Rapids, in the county of Linn and 5 State of Iowa, have invented certain new and useful Improvements in Size and Processes of Making Same, of which the following is a specification.

My invention relates to the manufacture 10 of a starch product for use particularly as a size in the textile industries; and the objects of the invention are to provide, first, a size or analogous product which will have certain novel and improved properties to be hereinafter described and claimed; and sec- 15 ond, an improved method of manufacturing a product of this character.

The invention is illustrated in the accompanying drawings which shows, diagrammatically in sectional elevation, a suitable apparatus for practising the process of my invention.

The purpose of sizing yarn, for example, in the manufacture of textile fabrics is to 25 strengthen the fabric and sometimes to give weight and body to it. The size penetrates and also coats the yarn, causing the fibers to adhere together. In order to give the size its capacity for penetrating the yarn I 30 produce a thin boiling starch of any desired degree of fluidity. The higher the degree of fluidity the greater will be the penetrating power of the size. In certain classes of fabrics, fabrics for example, that are 35 not ordinarily washed, it is important to have the size penetrate the yarn as completely as possible in order that the cloth should have weight and body. It is desirable also, under certain circumstances, that 40 the size should coat each of the fibers of the yarn in order to strengthen the same. I provide a size for accomplishing both these results by mixing with the thin boiling starch a certain amount of ordinary raw or 45 thick boiling starch. The thin boiling starch, because of its fluidity, penetrates the yarn. The thick boiling starch, because of its viscosity, cannot penetrate the yarn but instead forms a film or thin covering around 50 the same.

To make a size more adhesive and smoother in its character for certain uses, my invention contemplates an alkaline modification either of the thin boiling starch alone or 55 of the mixture of thick and thin boiling starches.

Furthermore, where desired, I introduce into the product, in such manner that it will be thoroughly diffused therethrough, other ingredients for example, a lubricating sub- 60 stance, such as petroleum oil, or other oil or fat; a hygroscopic substance, such as calcium chlorid; and any suitable germicide for preventing the size from spoiling. These ingredients may be considerably va- 65 ried, even omitted, without departure from my invention.

Finally, the product is reduced to a commercial form, for instance, to powder. In this form it may be shipped to the textile 70 mill and will only require mixing with water when it is to be used. In other words, the material sent to the mill is a complete size, the properties and characteristics of which will be varied during manufacture to 75 meet the requirements of the work in connection with which it is intended to be used, so that when the material reaches the user it will be ready for immediate use. No other substances need be mixed with it ex- 80 cept the water employed in reducing it to a usable liquid state.

Referring to the drawing, which illustrates apparatus for carrying out the preferred method of manufacturing this product, 1, 2 and 3 are vessels in which the starch is treated to suitably modify it. The raw starch is removed from the starch tables 4 and mixed with water in a breaker tank 5 which is provided with an agitator 6. From 90 the breaker tank the starch milk is run through a pipe 7 having branches 8, 9 and 10 into the treating vessels 1, 2 and 3. 11 is the acid tank and 12 the acid line running to the treating vessels. Heat is applied to 95 the material in the treating vessels to raise the material to a temperature safely below the gelatinization point, say to about one hundred and twenty degrees Fahrenheit, by means, preferably, of a hot water circulat- 100 ing system. The water is heated in a vessel 13 by means of a steam coil 14, water being supplied to the tank through pipe 15 and steam to the coil through pipe 16. The water from the tank 13 is circulated by a 105 pump 17 through pipe line 18 which is provided with branches or loops 19 arranged in the vessels 1, 2 and 3. Vessels 1 and 2 and vessels 2 and 3 are connected by valved pipes 20. 21 is a pipe connected by valved 110 branches 22 to each of the vessels. 23 is a pipe leading from pipe 21 over the vessels

and having valved branches or spouts 24 for delivering liquid into said vessels. By this arrangement of pipes an inter-circulation may be maintained between the treating vessels for the purpose of insuring perfect uniformity in the product. The circulation of the liquid is brought about by a pump 25. The course of the liquid will depend upon the adjustment of the valves in the piping just described. The liquid may, for example, be drawn from vessel 3 through pipe 21 (in which case valve 22 of vessel 3 will be open and the corresponding valves of vessels 1 and 2 closed) and introduced into vessel 1 through pipe 23 and the branch pipe 24 which leads to vessel 1, the valves in the other branch pipes 24 being closed. In such case the valves in the pipe 20 will be open so that the liquid in the vessels will equalize through these pipes. The treating vessels 1, 2 and 3 are preferably provided with agitators 26 which are kept in revolution by any suitable mechanism (not shown). When the starch has been modified to produce thin boiling starch of the desired fluidity, say to a fluidity of sixty degrees or above, depending upon the character of the product desired, the thin boiling starch may be run through the filter presses 27 and vacuum drier 28 and treated as hereinafter described. Where, however, it is desired that the product have the capacity for coating the yarn as well as penetrating it so that it will give the yarn the maximum strength as well as weight, I mix with the thin boiling starch a quantity of thick boiling or ordinary table starch which may be taken from the starch tables 4, reduced to starch milk in the breaker tank 5 and run into the treating vessels through pipes 7, 8, 9 and 10. This starch is thoroughly mixed with the thin boiling starch by means of the agitators aided, preferably, by the inter-circulation between the vessels above described. In order to give the product additional adhesiveness and to make it smoother in its character the mixed thin and thick boiling starch is given further treatment with an alkali, for example, with caustic soda. Supposing that a product is required having a penetration represented by forty degrees fluidity, I produce a thin boiling starch having a fluidity of seventy-five degrees and mix with this table starch in the proportions of 80 parts table starch to 100 parts of thin boiling starch, by weight. The mixture is then treated with an alkali, the application of heat being unnecessary, using for example, one-tenth of one per cent. by weight of caustic soda. The resultant product will have approximately the desired degree of fluidity, namely, forty per cent. and it will be smoother in its character than material not subjected to the alkaline treatment. That is, the yarn when sized with the prod-

uct will not have the harshness observable in yarns treated with a size produced by the acid modification alone. The product, however, is not alkaline in its character. It still has a slightly acid reaction.

If penetration is the quality chiefly required in the size, the raw or thick boiling starch may be omitted and where the other qualities of smoothness and additional adhesiveness are desirable the thin boiling starch may be subjected to the alkali treatment. Thin boiling starch as well as raw starch is affected by the alkali and its fluidity decreased. It is necessary, therefore, to modify the thin boiling starch to an extent which will give it greater fluidity than is required in the finished product. The treatment to which the starch must be subjected will depend, of course, upon the capacity for penetration which is required in any given case. With the knowledge that the fluidity of thin boiling starch is decreased by alkaline treatment it is an easy matter to work out empirically the degree of fluidity which it is necessary to obtain in the starch before subjected to treatment with the alkali in order that a product should be obtained having the proper capacity for penetrating the yarn.

Referring to the drawing, 29 indicates the starch tank for the alkali and 30 the supply pipe therefrom which is provided with valved branches 31 leading to the treating vessels. The product from the converting vessels is run to the filter presses 27 through a pipe 32 connected by branch pipes 33 with the bottoms of the treating vessels and provided with a pump 34. A conveyer 35 is arranged under the filter presses and conveys the starch to a hopper 36 which discharges the same into the drier. Preferably I employ a vacuum drier 28. The product, when dried, is discharged into a hopper 37. If additional ingredients are to be added to the size this operation is preferably performed during the latter part of the drying step. For example, I may mix with the starch a certain amount of some lubricating substance, such as petroleum oil, animal fat, or the like, petroleum oil being preferred. It is also possible and desirable, under some circumstances, to mix a small amount of calcium chlorid with the material for the purpose of making it hygroscopic. In order to prevent the product from souring when wet up and kept for several days, it may include any suitable germicide. These ingredients, or such of them as are employed, are mixed together in liquid form in a storage tank 39 and are injected into the material in the vacuum drier by means of an atomizing device 40. The drier is preferably of the general construction shown diagrammatically in the drawing.

The cylindrical casing of the drier is pro-

vided with a steam jacket 41. Within the casing is a revoluble drum 42 through which steam is circulated. Secured to the drum are agitating blades 43. The atomized liquid is drawn into the drier by the vacuum produced therein. It is thoroughly mixed with the material in the drier by means of the agitators 43.

The product will be in the form of a dry powder. By "dry" I mean commercially dry, that is, containing approximately the percentage of moisture which is standard in starch products of this general class, that is to say, ten to fourteen per cent. moisture.

15 I claim:

1. A size containing thick boiling starch mixed with thin boiling starch.

2. A size containing starch modified by acid treatment and starch modified by treatment with an alkali.

3. A size containing thin boiling starch modified by acid treatment, thick boiling starch and starch modified by treatment with an alkali.

25 4. A dry sizing material containing modified starch and a lubricant intimately mixed together.

5. A dry sizing material containing modified starch, a lubricant and a hygroscopic substance intimately mixed together.

30 6. A dry sizing material containing modified starch, a lubricant and a germicide intimately mixed together.

7. A dry sizing material containing thick 35 boiling starch intimately mixed with thin boiling starch.

8. A dry sizing material containing thin boiling starch modified by an alkali.

40 9. A dry sizing material containing starch modified by acid treatment and starch modified by treatment with an alkali.

10. A dry sizing material containing a mixture of thin boiling starch and thick boiling starch modified by treatment with 45 an alkali.

11. A size in the form of a dry powder containing thick boiling starch mixed with thin boiling starch.

50 12. A size in the form of a dry powder containing thin boiling starch modified by treatment with an alkali.

13. A size in the form of a dry powder containing thin boiling starch and raw starch both modified by treatment with an 55 alkali.

14. The method of producing a sizing

material which comprises modifying starch with an acid under conditions which produce thin boiling starch, mixing thick boiling starch with the thin boiling starch, and 60 subjecting the mixture to treatment with an alkali.

15. The method of producing a sizing material which comprises modifying starch with an acid under conditions which produce thin boiling starch, and then treating 65 the thin boiling starch with an alkali.

16. The method of producing a sizing material which comprises modifying starch with an acid under conditions which produce a thin boiling starch having a degree 70 of fluidity greater than the fluidity required in the finished product, and then modifying the thin boiling starch by treatment with an alkali.

17. The method of producing a sizing material which comprises modifying starch with an acid under conditions which produce thin boiling starch having a fluidity greater than that required in the finished 80 product, mixing thick boiling starch with the thin boiling starch, and subjecting the mixture to treatment with an alkali.

18. The method of producing a sizing material which comprises modifying starch 85 under conditions which produce thin boiling starch, drying the product and during the drying operation intimately mixing a lubricating substance therewith.

19. The method of producing a sizing 90 material which comprises modifying starch under conditions which produce thin boiling starch, drying the product to a powder, and mixing a lubricating substance in atomized form with said powder.

20. The method of producing a sizing material which comprises modifying starch with an acid to make the starch thin boiling, and thereafter treating the same with a 95 caustic alkali.

21. The method of producing a sizing material which comprises modifying starch with an acid to make the starch thin boiling, and thereafter treating the same with a caustic alkali in an amount insufficient to 100 give the product an alkaline reaction.

22. The method of producing a sizing material which comprises modifying starch with an acid to make the starch thin boiling, then mixing in raw starch and treating the 110 mixture with a caustic alkali.

ADOLPH W. H. LENDERS.